

## UNITED STATES PATENT OFFICE

2,635,323

## NONCURLING FABRIC

Heinz Ginzel, Dornbirn, Vorarlberg, Austria

No Drawing. Application July 11, 1947, Serial  
No. 760,512. In Germany November 19, 1942Section 1, Public Law 690, August 8, 1946  
Patent expires November 19, 1962

9 Claims. (Cl. 28—78)

1

This invention relates to non-curling, chemically stiffened fabrics, the textiles produced therefrom and a method of producing such fabrics and textiles.

Chemically stiffened fabrics, made of native or regenerated cellulose, particularly those highly improved and stiffened by a treatment with concentrated mineral acids, as sulphuric acid, or with other hydrolysing and/or swelling agents, as zinc chloride, calcium thiocyanate, ammoniacal copper oxide or with mercerising lye at low temperatures, often have the disagreeable quality of curling when dried or ironed. Such a tendency to curl exists with fabrics chemically stiffened on the whole surface or a large part of their surface, especially in cases where the stiffened portions form a connected ground. It has been recommended that the curling tendency may be avoided by passing the parchmentized material through successive jaws of a calender having at least two jaws. A permanent suspension of the curling tendency of parchmentized fabrics could however not be obtained by this process. According to a later proposal for obtaining non-curling parchmentized or otherwise chemically permanently stiffened fabrics, fabrics the warp or weft of which or both woven by means of normally right-hand and left-hand twisted yarns interspersed therein, for example, alternating individually or in groups, that is to say yarns twisted alternating in different directions are subjected to parchmentizing or an equivalent stiffening process. This latter process needs special measures in spinning and weaving because the working up of yarns twisted in different directions makes it necessary to dye the different yarns with different colors, which colors have to be removed after weaving and also the production of the fabrics requires special precautions.

An object of this invention is to provide chemically stiffened cellulose containing fine fabrics, and more particularly an organdie, permanently free from a curling tendency. Another object of this invention is to provide a simple method which makes it possible to produce parchmentized fine fabrics, which are free from inner tensions without being passed through successive jaws of a calender and which keep permanently a non-curling character. Other objects of this invention will appear as the description proceeds.

According to this invention chemically stiffened cellulose containing fine fabrics consist of threads (yarns or twines) twisted in one direction only, having an English yarn number over 60, and more particularly at least 80, the warp and the weft being substantially equal in weight.

The invention is based on the new recognition that the curling tendency of chemically improved, stiffened fabrics is a function of the distribution of the weights of warp and weft. While

2

parchmentized fabrics, made of the usual fine fabrics, show a well known very large curling tendency, the coarser fabrics, which are treated with concentrated sulphuric acid to provide an imitation linen, do not show this tendency. It was first suggested that the curling tendency in the coarse fabrics had been suspended by the strength of the threads, but this has been proved to be wrong. Further investigations have shown that the absence of the curling tendency of the coarse fabrics is a result of their structure. Such comparatively coarse fabrics usually have a square or nearly square structure, as these fabrics contain approximately the same number of yarns in one unit of length of weft and warp, and the yarns of weft and warp have the same strength, measured by the yarn number. Such coarse fabrics are for instance fabrics with a set of 21/21 and an English yarn number of 30/30, or a set of 16/16 and an English yarn number of 20/20. The set is the number of threads or yarns in the warp and weft in  $\frac{1}{4}$  Paris inch (6.767 mm.), and the English number indicates how many hanks of 840 yards (768.10 m.) weigh one pound (453.59 g.), so that a higher number indicates to a finer yarn. In contradistinction to the structure of such coarse fabrics used for the imitation of linen, there are used for the production of chemically stiffened transparent fine fabrics mainly raw fabrics with a set of 24/21 and an English yarn number of 80/120. With the usual fine fabrics, used for parchmentizing, the set, i. e. the number of threads in the warp on the one hand and in the weft on the other hand is more unequal than with the coarse fabrics, but, more importantly, the strength of the yarns measured by their yarn numbers is very different in weft and warp. Experiments have now shown that fine fabrics with a yarn number of more than 60, particularly 80 and more, for instance 100, 130, 180 etc., do not curl after parchmentizing or other chemical stiffening, if the original fabrics were set approximately square, that is with the same number of threads and the same yarn numbers in weft and warp. The reason is, as was proved, the approximate equality of weight of weft and warp in a unit of area (for instance one m.<sup>2</sup>) with such "square" set fabrics. It may be seen that the expressions

$$\frac{Ew}{Nw}$$

and

$$\frac{Ef}{Nf}$$

wherein E is the number of threads per unit of area (for example, in a square meter), N is the English yarn number, a w and f designate warp and weft, respectively, represent values which are

proportional to the weight of the warp and the weft, respectively, in the unit of area, since the English yarn number is inversely proportional to the weight of thread per unit of length. Approximate equality between these expressions will, accordingly, indicate the presence of the conditions necessary to avoid curling of the parchmentized fine fabric.

In accordance with this finding that the crucial point is the equilibrium of weight between weft and warp, it was concluded that "unsquare" set fine fabrics also should be free of a curling tendency after parchmentizing if the fabric contains approximately the same weight of weft and warp in one unit of area, for instance a smaller number of stronger weft threads and a larger number of weaker warp threads. This has indeed been proved by experiments. A small deviation from the equilibrium of weight does not largely influence the success. Generally a difference up to 10%, more particularly a difference of not more than about 7%, between the weights of weft or warp and half of the weight of the fabric is allowable without causing a considerable tendency towards curling. The nearer the weights of weft and warp come to half of the weight of the fabric, the more the tendency to curl is prevented.

It has also been found that the manner of chemical treatment, especially the degree of shrinkage resulting from parchmentizing or other chemical stiffening is without essential importance, because due to the shrinking of stronger yarns in the warp, the number of unshrunken yarns in the weft will rise proportionally, and vice versa, so that the shrinking will result in an increase in weight of one unit of area of the fabric, but the relation of the weights of warp and weft will remain nearly constant. As well, the relation between the weights of warp and weft remains constant in the case of shrinking in both directions.

The fabrics produced in accordance with this invention may be stiffened by any chemical process producing a permanent stiffening effect such as parchmentizing or transparentizing with mineral acids, particularly with highly concentrated sulphuric acid or other parchmentizing agents, as ammoniacal copper oxide solution, zinc chloride, calcium thiocyanate and so on, or by treatment with mercerising lyes at low temperatures, the concentration, temperature and time of such treatments being adjusted in a way known, corresponding to the material to be treated. The stiffening may be carried out in combination with shrinking or stretching the

surfaces in the form of a pattern, or by other equally well known methods.

Preferably, fine textiles of cotton or regenerated cellulose, as artificial silk or rayon (viscose, copper cellulose or acetate silk or wool) are employed in the practice of this invention. The fabrics may contain fancy threads of the same or other materials, or instance animal fibres or synthetic fibres, as polyamide fibres, glass fibres, metal fibres, metalized fibres, and so on. The fabrics also may contain corrosive threads or yarns, which may be removed before, during, or after the chemical stiffening process by one of the known wet or dry etching processes. The fabrics consist of uni-directionally twisted threads, i. e., they consist of either right-hand or of left-hand twisted threads. Standard twisted yarns as well as crepe yarns may be used.

The invention offers the advantage of providing non-curling, chemically stiffened, preferably parchmentized fine fabrics, which may be produced without using complicated measures, as the use of yarns twisted in different directions and also without special weaving equipment. Another advantage is that the tensile strength and the resistance against rubbing are nearly equal in both directions (weft and warp) with a final product of square structure. These qualities also prevail with textiles produced of such fabrics, as decorative clothes, trimmed products, collars, jabots, ruches, ladies' dresses, blouses, decorative aprons and the like.

The following examples will further illustrate the nature of this invention.

The chemical stiffening of the cotton fabrics was accomplished under the same conditions in all experiments. The fabrics were premercerised with a sodium hydroxide solution of 27° Bé. for 30 seconds while shrunk in breadth, were bleached and then parchmentized with sulphuric acid of 54° Bé. for 8 seconds at a temperature of 0° C. The following fabrics were used:

TABLE A

Original fabrics

|    | a | b   | c     | d       | e     | f     | g    | h     | i    |
|----|---|-----|-------|---------|-------|-------|------|-------|------|
| 50 | 1 | 120 | 24/21 | 80/120  | 26.2  | 15.3  | 41.5 | 20.75 | 26.5 |
|    | 2 | 120 | 25/26 | 180/180 | 12.1  | 12.6  | 24.7 | 12.35 | 22   |
|    | 3 | 115 | 24/22 | 100/100 | 21.0  | 19.2  | 40.2 | 20.10 | 44.4 |
|    | 4 | 115 | 24/21 | 100/100 | 21.0  | 18.4  | 39.4 | 18.70 | 6.7  |
|    | 5 | 120 | 26/32 | 130/160 | 17.40 | 17.40 | 34.8 | 17.40 | 30   |
|    | 6 | 120 | 22/27 | 130/160 | 14.8  | 14.8  | 29.6 | 14.8  | 30   |

TABLE B

Fabrics after the chemical stiffening

| a  | b   | c       | d       | e    | f    | g    | h     | i    |                    |
|----|-----|---------|---------|------|------|------|-------|------|--------------------|
| 1a | 98  | 29/21   | 80/100  | 31.6 | 18.3 | 49.9 | 24.95 | 26.5 | intensely curling. |
| 1b | 110 | 26/21   | 80/110  | 28.3 | 16.6 | 44.9 | 22.45 | 26.5 |                    |
| 2a | 98  | 30.6/26 | 180/147 | 14.3 | 15.4 | 30.2 | 15.10 | 2.0  |                    |
| 2b | 107 | 28/26   | 180/169 | 13.6 | 14.2 | 27.8 | 13.00 | 2.0  |                    |
| 3  | 112 | 24.6/22 | 100/97  | 21.5 | 19.7 | 41.2 | 20.60 | 4.4  |                    |
| 4  | 112 | 24.6/21 | 100/97  | 21.4 | 18.8 | 40.2 | 20.10 | 6.7  |                    |
| 5  | 98  | 32/32   | 130/130 | 21.4 | 21.4 | 42.8 | 21.4  | 0    | Do.                |
| 6  | 98  | 27/27   | 130/130 | 18.1 | 18.1 | 36.2 | 18.10 | 0    |                    |

fabric in length or in breath. The fabrics may be treated before, during or after the stiffening in any desired way, for instance they may be mercerised, bleached, dyed or printed.

The invention may be applied to fabrics stiffened on the whole of their surfaces or stiffened locally only on parts of the surfaces, the latter being effected by printing stiffening agents on the

In the preceding tables:

Column a, indicates the series number of the experiment; column b, the breath of the fabric; column c, set (number of threads in 1/4 Paris inch); column d, English number of yarn (the first number in columns c and d refers to the warp and the second to the weft); column e, weight of one m.<sup>2</sup> of warp in g; column f, weight

of one m.<sup>2</sup> of weft in g; column g, total weight of one squaremeter; column h, half of the weight of one squaremeter of the fabric; and column i, difference in weight of warp or weft from value h in percent.

These tables prove, that the fine fabrics, generally used for chemical stiffening (Examples 1 of the tables) show a very large deviation of weight of the weft of the warp amounting to 26 or 27% in both directions from the equilibrium of weight (half of the total weight of the fabric). Such fabrics roll strongly after stiffening.

In contrast thereto the fabrics according to the Examples 2 to 6 do not have any tendency towards curling. Those fabrics have approximately the same weights of weft and warp, the deviation from the equilibrium of weight in the Examples 2, 3 and 4 being only 2.0%, 4.4% and 6.7% respectively, while fabrics according to the Examples 5 and 6 are completely in equilibrium as to the weights of warp and weft.

The Examples 2 to 4 demonstrate an embodiment of the invention with the use of approximately square set fabrics (fabrics with about the same number of threads and equal strength of threads in weft and warp). The Examples 5 and 6 show an embodiment of the invention with the use of unsquare set original fabrics, the final products showing an approximately square set. The comparison of the examples proves that the crucial point in removing the tendency to curl is the maintenance of the substantial equality of weight between weft and warp. The Examples 1a, 1b, 2a, 2b (Table B) prove further, that the degree of shrinkage produced by the finishing has no decisive influence on the curling tendency.

I claim:

1. An organdie consisting of parchmentized threads twisted in one direction only, said threads having an English yarn number over 60, the weight of the warp and the weight of the weft of the organdie in a unit of area each being within 10% of one-half of the total weight of the said unit of area.

2. An organdie consisting of parchmentized threads twisted in one direction only, said threads having an English yarn number of at least 80, the weight of the warp and the weight of the weft of the organdie in a unit of area each being within 10% of one-half of the total weight of the said unit of area.

3. An organdie consisting of parchmentized threads twisted in one direction only, said threads having an English yarn number over 60, and the weight of the warp and the weight of the weft

of the organdie in a unit of area being substantially equal.

4. An organdie according to claim 3 in which the threads are parchmentized at certain defined areas and not parchmentized at other defined areas.

5. An organdie consisting of parchmentized threads twisted in one direction only, said threads having an English yarn number greater than 60, in which organdie

$$\frac{Ew}{Nw}$$

and

$$\frac{Ef}{Nf}$$

differ by less than 10% from one another, Ew being the number of warp threads in a unit of area, Ef being the number of weft threads in the same unit of area, and Nw and Nf being, respectively, the English yarn number of the warp threads and the weft threads.

6. An organdie as claimed in claim 1 in which the threads are parchmentized at said defined areas and not parchmentized at other defined areas.

7. An organdie as claimed in claim 2 in which the threads are parchmentized at said defined areas and not parchmentized at other defined areas.

8. An organdie consisting of parchmentized threads twisted in one direction only, said threads having an English yarn number of about 80, the weight of the warp and the weight of the weft of the organdie in a unit of area each being within 7% of one-half of the total weight of the said unit of area.

9. An organdie as claimed in claim 8 in which the threads are parchmentized at certain defined areas and not parchmentized at other defined areas.

HEINZ GINZEL.

45 40 45 References Cited in the file of this patent

UNITED STATES PATENTS

| Number    | Name        | Date           |
|-----------|-------------|----------------|
| 2,215,938 | Schonholzer | Sept. 24, 1940 |
| 2,249,039 | Platt       | July 15, 1941  |
| 2,400,182 | Whitman     | May 14, 1946   |

OTHER REFERENCES

55 "Staple Cotton Fabric," Hoye, published 1942, McGraw-Hill Book Co., New York, pages 57, 58 and 60.